

March 3, 1936.

B. W. SMITH

2,032,816

METHOD OF MAKING SAFETY PAPER

Filed Aug. 25, 1932



INVENTOR  
BURGESS W. SMITH

BY *Edward H. Cumpston*

ATTORNEY



## UNITED STATES PATENT OFFICE

2,032,816

## METHOD OF MAKING SAFETY PAPER

Burgess W. Smith, Rochester, N. Y., assignor to  
 The Tedd Company, Inc., Rochester, N. Y., a  
 corporation of New York

Application August 25, 1932, Serial No. 630,451

5 Claims. (Cl. 91—67.95)

This invention relates to methods of making safety paper for paper forms, instruments, and other documents requiring protection against fraudulent alteration, and, more particularly, to the variety of safety paper embodying means adapted to be rendered operative on the application of chemical eradicators, to warn of attempted alteration. One object of the invention is to provide a more simple and economical method of manufacturing such paper.

Another object is the provision of such a method capable of producing paper of white or uniformly tinted color, or having any desired pattern on it.

Another object is to provide a simple and inexpensive method of the character described, adapted for making paper containing an inherently warning word or other symbol, of an initially illegible character, but applied in a material which is reactive to chemical eradicating substances so as to develop a conspicuous color or stain upon the use of such substances in attempting alteration.

A further object is the provision of a method of the character described in which the warning symbol is applied to the paper in an initially illegible form but incorporated in the body of the paper itself, in a manner rendering it accessible to the eradicating substances, so as to secure conspicuous and permanent development of the warning color or stain.

To these and other ends the invention resides in certain method steps and combinations of steps, all as will be hereinafter more fully described and pointed out in the claims at the end of the specification.

In the drawing:

Fig. 1 illustrates, diagrammatically, one form of equipment for practicing the invention; and

Fig. 2 illustrates in a general way one form of safety paper which may be produced by the invention.

It has been proposed heretofore to make safety paper by printing on it, before or after sizing, a pattern or symbol, with a colorless chemical or ink capable of reacting with chemical eradicators to develop a warning color or stain. It has been found, however, that the most efficient sensitive or developing chemicals for this purpose are generally of a more or less water soluble nature so that it has not been found practicable to apply such chemicals to the paper during the formation of the same or prior to sizing because of the tendency of such chemicals to be dissolved and removed from the paper. It has been found, on the other hand, that the application of such

warning symbols to the paper after sizing, by the usual methods of printing, produces such a disturbance of the surface of the paper that such symbols are initially legible because of the difference in the light reflecting action of the paper surface, as between the printed and unprinted portions, particularly in certain angles of incidence of the light, with the result that such initial legibility of the warning symbols renders the paper unsuitable for use.

My prior Letters Patent, Nos. 1,454,837, 1,675,769, and 1,689,302, describe and claim methods of making safety paper in which the initial illegibility of the warning characters is insured by the use of a camouflaging pattern. 15 My Letters Patent, No. 1,817,171, discloses and claims a further method of making such paper to reduce the legibility of the warning characters where no camouflaging pattern is employed.

My present invention provides a further simple and inexpensive method for producing such paper, having various other advantages such as increased initial illegibility of the warning symbols, the penetration of the sensitive chemical or ink into the paper to resist removal by abrasive methods, as well as accessibility to the action of eradicating chemicals to insure rapid and thorough development of the warning color or stain, as well as being generally available for making safety paper of various kinds and styles. 30 In accordance with the present invention it has been found that these advantages may be accomplished by printing the warning symbols on the paper after the sizing bath, while the paper is still moist or by moistening the formed paper 35 before printing. It has been found that by so printing on the moist paper with a chemical or ink that is miscible with water, or which contains dispersed therein active material soluble in water, it is possible to use a minimum of pressure, so as not to indent the paper. As more fully described below a suitable sensitive chemical or ink is employed of a substantially colorless nature, after the application of which the paper is dried and finished, with the result that 45 the chemical penetrates the paper and its presence is further obscured by the finishing operations, so that it becomes completely invisible.

One variety of equipment or apparatus by which the invention may be produced is illustrated schematically in Fig. 1 of the drawing in which 10 represents a supply roll of the paper web 12 passing under a roll 13, immersed in water or its equivalent in a vat 25, from which the web is carried through squeeze rolls 14 and 15 to re- 55

move the surplus liquid. The web may then be passed directly to the printing rolls, hereafter described, but is preferably immersed a second time in the vat 25 under a roll 18 from which it proceeds through a second pair of squeeze rolls 17 and 18 which remove all but a trace of the liquid from its surface.

From the bath in vat 25 the web then goes between a print roll 19 and an impression roll 20 and thence to suitable drying and finishing appliances. The print roll 19 is engraved with warning indicia, such, for example, as the words "Void" and "Fraud", and is inked by the rubber or composition rolls 21 and 21' which in turn receive a supply from the roll 22 supplied from the fountain 24 by means of an oscillating roll 23. This inking mechanism may have the usual or any suitable arrangement in accordance with the known construction commonly employed in printing presses.

In the vat 25 through which the paper passes as described on the way to the printing device, I have used water without the admixture of any substances, or a size adapted for the purpose, or I may use a colored bath of dye, or size containing the same, which will color the surface of the paper in a uniform tint where the rolls 14 and 15, or 17 and 18, in case the latter are used, have plain or smooth surfaces. Should either pair of squeeze rolls be engraved with a pattern or design, such pattern or design will be impressed upon the paper in the manner described in Letters Patent to LaMonte and Saxe, No. 123,782. Such steps provide an economical and continuous method of marking the paper with a plain tint or color design or pattern, respectively, after which the paper so marked may be passed to the printing devices to there receive an invisible printing of the warning symbols in a suitable chemical or ink applied to the roll 19 by means of the mechanism described above.

A suitable, substantially colorless sensitive chemical or ink for applying the warning symbols by means of the roll 19 is fully described in my copending application Serial No. 512,196, filed January 29, 1931, namely, a material comprising diphenol and diphenyl-guanidine or related substances as described in said co-pending application. Conditions may make it desirable to use glycerine or similar hydroscopic material to prevent the chemical or ink from drying on the inking and printing rolls, as well understood in the art. I may also use such compounds as 1,3,5, aminomethylchlorobenzothiazole, which may be in the form of the base, sulphate, hydrochloride or other salt dissolved or dispersed in a water-miscible medium, such as a solution of gum arabic in glycerine. It may also be ground into a varnish comprised of sulphonated oil, such as Turkey red oil. Such inks are substantially colorless and stable until reaction with a chemical eradicator with which they develop a conspicuous color or stain of a permanent nature difficult to remove.

From the printing rolls 19, 20, the paper web is preferably passed through drying rolls 26 and thence to a calender stack 27 and subsequently rewound in a roll 28. Instead of the calendering with rolls 27 some other form of finishing may be employed for removing any disturbance caused by printing of the homogeneous condition of the paper surface.

While it is practicable to print, dry, and finish the paper containing the warning symbols in a continuous operation as described, there are cer-

tain advantages to be gained by rewinding the paper while moist after receiving the impression from the printing rolls 19, 20 and allowing it to stand, so that the sensitive ink will penetrate into the body of the paper, in order that its removal, by abrasive treatment, will so reduce the thickness as to make such treatment readily discernible.

The application of a water-miscible chemical or ink to the moist paper by the separately inked printing roll 19 has the effect of causing the warning symbol thus printed to be so diffused into the body of the paper that the outline of the letters of the warning word or symbol are blurred, instead of being sharp, which further reduces any tendency to initial legibility of the printing due to any slight color the ink may have. The described method further makes it possible to use a minimum of foreign matter in the preparation of the ink so that the active material is more easily acted upon by the chemical eradicator, thus increasing the rapidity and depth of color development. It will be seen that the above method is far more economical than the application of the sensitive chemical or ink to the paper by addition, for example, to the beater or to a bath in which the paper is submerged, since the sensitive chemical or ink is generally of a more or less expensive character, especially in a pure state and good quality and since, by the present method, it is substantially all applied directly to the paper at those portions only desired to be treated with it. The final calendering or other finishing operation removes any disturbance of the surface condition of the paper and affords a uniform and homogeneous appearance which completes the application of the warning symbols in a completely illegible manner.

The contents of vat 25 may include a coloring substance which is fugitive under the action of chemical eradicators or itself develops a warning color or stain in reaction therewith, as well understood in the art, and by providing one of the rolls 14, 15, or 17, 18 with a desired design or pattern, the method may be advantageously employed to produce, instead of a uniformly white or tinted paper, a paper combining with the warning symbols a surface pattern adapted to protect against mechanical erasure or to ornament the paper.

By the terms "colorless" or "substantially colorless" I mean that the warning words on the paper when finished will not be readable, and if the strength of the printing is sufficient to be readily readable when activated by an ink eradicator, the intention of the terms is correct.

I claim:

1. The method of producing safety paper comprising wetting said paper with a solution of a dye, pressing said paper between a pair of rolls one of which has its surface formed with a pattern to mark the paper and remove the surplus solution, printing from a separately inked surface a warning symbol on the surface of said wet paper with a water-miscible ink other than said dye, which ink is initially illegible and contains a substantially colorless compound adapted to be darkened by the action of an ink eradicator, and drying and finishing the paper surface so that said warning symbol is not readable.

2. The method of producing safety paper comprising wetting said paper with a solution of a dye, pressing said paper between a pair of rolls one of which has its surface formed with a pat-

tern to mark the paper and remove the surplus solution, printing from a separately inked surface a warning symbol on the surface of said paper while moist and substantially without pressure with a water-miscible, initially illegible ink other than said dye containing a substantially colorless compound adapted to be darkened by the action of an ink eradicator, allowing said paper to stand for a substantial period to absorb said ink, drying said paper, and finishing its surface so that said warning symbol is not readable.

3. The method of producing safety paper comprising moistening the paper with water or a water solution, printing a warning symbol on the moistened paper with a printing surface separately inked with a water-miscible ink other than the substance with which said paper is moistened, which ink is initially illegible and contains a compound adapted to be discolored by the action of the chemical eradicator, and drying and finishing the paper, so that said warning symbol is not readable.

4. The method of producing safety paper comprising moistening said paper with water or a

water solution, printing a warning symbol on said moistened paper without substantial pressure by means of a printing surface separately inked with a water-miscible ink other than the substance with which said paper is moistened, which ink is initially illegible and contains a compound adapted to be discolored by the action of ink eradicators, allowing said paper to stand for a substantial period to absorb said compound, and then drying the paper and finishing its surface, so that said warning symbol is not readable.

5. The method of producing safety paper comprising moistening said paper with a water solution of a dye, removing the surplus solution, printing a warning symbol on said moistened paper substantially without pressure by means of a printing surface separately inked with a water-miscible ink other than said dye which ink is initially illegible and contains a substantially colorless compound adapted to be discolored by the action of an ink eradicator, drying said paper, and finishing the paper surface, so that said warning symbol is not readable.

BURGESS W. SMITH.